

## UNITED STATES PATENT OFFICE

2,291,061

## METHOD OF IMPROVING THE DYEING PROPERTIES OF ARTIFICIAL TEXTILE MATERIALS

Paul Schlack, Berlin-Treptow, Germany, assignor, by mesne assignments, to Walther H. Duisberg, New York, N. Y.

No Drawing. Application February 17, 1939, Serial No. 256,857. In Germany February 11, 1936

5 Claims. (Cl. 8—129)

My present invention relates to improving the dyeing properties of artificial threads, especially acetate rayon threads.

This application is a continuation in part of my application Ser. No. 123,868 filed February 3, 1937.

I have proposed (U. S. Patent No. 2,131,145) to modify more or less profoundly, especially in respect of affinity and fastness to dyestuffs, the chemical character of textile materials which consist of or contain protein substances or derivatives or conversion products thereof by action of an alkyleneoxide or a derivative or analogue thereof which may contain in addition to the reactive heterocyclic ring a basic or an acid group, for instance ethyleneoxide, 1:2-propyleneoxide, epichlorhydrin, piperido-propenoxide, 1:2-propylenesulfide, 1-chloro-2:3-propylenesulfide, N-butyl-ethyleneimine, N-diethyl ethylene iminium chloride, sodium-2:3-epoxyp propane-1-sulfonate.

During this reaction substitution occurs at the basic as well as at the acid groups, coupled with a shifting of the iso-electric point or region. In most cases the absorption capacity for acid dyestuffs is increased and that for basic dyestuffs diminished, however, the conditions may be changed completely if the substituting residues contain acid groups, especially sulfo-groups.

I have also shown (U. S. Patent No. 2,131,146) that textile materials of protein substances and other basic materials of high molecular weight, which contain residues capable of being alkylated, may be converted in a similar manner and with similar results with mixtures of alkylene oxide and the reactive alkyl ester of an inorganic or an organic-inorganic acid. Finally, I have recommended (U. S. Patent No. 2,131,121), that textiles, which contain basic residues attached to natural or artificial polymeric bodies, and which are dyed with acid dyes should be after-treated with alkyleneoxides or derivatives or analogues thereof for the purpose of improving the fastness of the dyeing.

Especially strong effects of this type, which may be connected with a decrease of the swelling capacity in an alkaline medium, are obtained by means of polyfunctional compounds of the type of epichlorhydrin.

In the U. S. Patent No. 2,097,120 it has further been proposed to introduce nitrogen into viscose rayon by treating the same with ethyleneimine. If necessary the treatment may be repeated several times.

My present invention has for an object to

provide a method of improving the dyeing properties of cellulose organic ester silk, and particularly of cellulose acetate rayon, which contains incorporated and fixed therein a certain amount of basic-reacting groups capable of being alkylated.

A further object of the invention consists in the provision of improved fibers of the kind referred to, which may be more easily and fastly dyed than cellulose ester threads, which have merely been subjected to a process, by which basic groups are introduced thereto.

Still further objects of the invention will appear as the following description proceeds.

The method of the invention consists in treating artificial textile materials produced from organophilic organic esters of cellulose, which textile materials contain incorporated and fixed therein basic groups, with an alkyleneimine, -oxide, or -sulfide before dyeing the same with an acid dye.

(The term "organophilic" denotes compounds which are soluble or at least capable of swelling strongly in organic solvents.)

The organic ester silk may contain a basic radical linked to the molecule chemically for instance the reaction product of cellulose derivatives with halogen alkylamines, halogen hydroxyalkylamines, ethylene imines and ethylene imine derivatives, or substituted aminopropenoxides.

It may furthermore contain an additional component for instance a resinous basic component. Examples of such additional components are basic substituted polymerizes, for example of the polyvinyl alcohol or polyacrylic acid series, for instance the reaction product of polyvinyl alcohol with halogen alkylamines, the condensation products of polyacrylic acid methyl ester and aliphatic polyamines, such as  $\beta$ -diethylaminoethylamine; also basic aldehyde resins, for example basic toluene arylsulfamide resins, basic phenol aldehyde resins, or basic alkyde resins.

A number of such resins are for instance described in the applications Ser. No. 47,638 filed October 31, 1935, and Ser. No. 64,776 filed February 19, 1936, Patent No. 2,183,754.

In the case of basic phenol resins as additions the treatment with the alkylene oxide has the particular advantage that it often improves essentially the stability of the product to light.

By the action of the alkylene oxides, -imines and -sulfides the reactivity of the textile materials particularly the affinity for dyestuffs, is considerably modified so that various effects become possible. Depending upon the selection of the

reactant, the affinity to acid or the affinity to basic dyestuffs or textile assistants may be influenced in the desired sense. Quite apart from the greater range in the choice of dyestuffs and dyeing processes which is obtained by the invention, in many cases a considerable improvement in the fastness of the dyeings to water, washing, milling, sweat, is produced.

With cellulose acetate rayon, which contains basic reacting groups the process of the invention is of especial advantage. The treatment with an alkylene imine for instance produces a very slight saponification and thus causes the formation of extremely fine pores in the hydrophobic substratum, thus facilitating the access of dyestuffs of considerable molecular dimensions, such as for instance chrome dyes to the basic groups or to the additional resinous components which contain such basic groups. I have found e. g. that a cellulose acetate, which contains an addition of a basic resin, and which may be dyed quite well with an ordinary simple acid wool dye, does not take up dyes of a more complicated structure, such as chrome dyes. Since these latter, however, yield the fastest dyeings, their employment represents a great advantage. The same cellulose acetate, if treated according to the process of the present invention before dyeing, takes up dyes of high molecular dimensions and of completed structure easily and fixes them fastly.

For the purpose of the invention there may be used a large number of substances belonging in a narrow and in a wide sense to the class of alkylene oxides and their derivatives and having the property of alkylating the compound containing the reactive group while splitting the heterocyclic ring. For example the following may be named: Ethylene oxide, propylene oxide, butylene oxide, cyclohexene oxide, phenoxypropenoxide, butadiene dioxide, glycidic, epichlorhydrin, epibromhydrin, epi-iodohydrin, 1-2-propylene - sulfide, 3-chlor-1,2-propylenesulfide, ethylene imine, N-butylethylene imine, N-diethylethylene iminium chloride, N-pentamethylene ethylene iminium chloride, the biquaternary spirocyclic compound from di- $\gamma$ -chlor- $\beta$ -hydroxypropylpiperazine. The reactive substances, so far as they are sufficiently volatile, may with advantage be used in the form of their vapors, generally at diminished or raised pressure. Less volatile substances are used in aqueous treating liquors, padding solutions or printing pastes or dissolved in organic solvents as for instance alcohol, acetone, carbontetrachloride, butanol, toluene, gasoline. The reaction may be accelerated by catalysts, for example salts, particularly halides, for instance sodium chloride, calcium chloride, trimethyl ammonium chloride, dodecyl trimethylammonium chloride or by bases, in some cases also by acids or acid reacting salts such as aluminium chloride or zinc chloride. If desired the catalyst may be applied only locally or in the form of a pattern, whereby pattern effects may be produced. Also the presence of condensing agents, especially of carbonyl compounds and derivatives thereof may be of advantage.

The working conditions to be observed from case to case as regards temperature, concentration of the reacting substances, time of reaction are dependent on the reactivity of the agents employed, on the capacity and degree of swelling, on the pH-value and on other influences, particularly also on the degree of dryness of the tex-

tiles. Of course the working conditions have to be adapted to the fastness of the substratum to chemical agents. For the gaseous treatment a suitable adjustment of the relative air moisture is sufficient. Therefore, it is necessary to find the most suitable working conditions for each case by simple experiments. With reactive compounds, for instance epichlorhydrin, ethyleneimine and the like a medium temperature between 40° and 80° and a time of reaction of 2 to about 16 hours will be necessary. Further details will be disclosed by the following examples.

(1) Acetate artificial silk which contains 10 per cent of the basic resin obtainable from polyacrylic acid ethyl ester and an equimolecular proportion of  $\beta$ -diethylamino-ethylamine at 120° to 130° C. (French Patent No. 798,460) after rinsing with dilute acetic acid and drying is heated at 92 per cent relative moisture at 80° C. with 20 per cent of vapor of epichlorhydrin for 15 hours.

The affinity to many acid-dyestuffs especially to such which previously were only badly absorbed as for instance to alizarincyaningreen, is considerably increased and also the fastness to washing of the dyeings is improved.

(2) Acetate artificial silk which contains 7.5 per cent of a basic resin made by heating dimethylaminoethanol with a novolak from 10 mol phenol and 7 mol formaldehyde in alcohol is treated for 12 hours at 80° C. with 10 per cent of epichlorhydrin and 10 per cent of ethylene oxide at 92 per cent relative moisture. Dyeings on the silk with acid dyestuffs, for instance Alizarine Direct Blue A (Schultz Farbstofftabellen 7th edition, vol. II, page 7) have a better fastness than they have on material which has not been pretreated in accordance with the example. The fiber also shows a smaller tendency to yellowing.

(3) Diethylaminoethyl cellulose made by the reaction of alkali cellulose and  $\beta$ -chlorodiethylamine is acetylated. Threads made from this acetyl-aminoethyl cellulose are pre-treated with very dilute hydrochloric acid and then washed with water and treated with 20 per cent of epichlorhydrin for 15 hours at 80° C. The dyeing properties of the material are improved, for instance dyestuffs of the type of Alizarincyaningreen G Extra (Schultz Farbstofftabellen, 7th edition, vol. I, page 532) are absorbed in greater quantities and the dyeings obtained are faster.

The affinity is enhanced if instead of hydrochloric acid, sulfocyanic acid is used or if an intermediate treatment with a salt of the sulfocyanic acid takes place. Instead of epichlorhydrin, 3-chloro-1,2-propylene sulfide may be used.

(4) An acetate artificial silk containing 8 per cent of the product obtained by reacting chlorinated hard paraffin with superfluous ethylenediamine is stored in a closed vessel (volume 40 cc. per 1 gram of textile fiber) in vapor of 10 per cent ethylenediamine for 8 hours at 70° C. at 45 per cent relative air moisture. Subsequently it is acidified with acetic acid (3 grams per liter) at 60° for  $\frac{1}{2}$  hour. The artificial silk treated in such a manner is dyed intensively with Alizarincyaningreen G Extra (Schultz Farbstofftabellen, 7th edition, vol. I, page 532) and similar acid dyestuffs. The dyeing is of good quality as regards the fastness. The fiber not after-treated with imine absorbs Alizarincyaningreen G essentially weaker.

(5) An acetate artificial fiber which contained 12 per cent of the mixed polymerizate from 1 mol maleic acid anhydride and 1 mol vinylmethylether

and which immediately after the spinning process is aminated by an after-treatment with a 3 per cent solution of 3-dimethylamino-1-amino-propane in trichlorethylene is stored in a closed chamber (volume 50 cc. per 1 gram of fiber) in 5 vapor of 12 per cent epichlorhydrin for 14 hours at 75° C. and 75 per cent relative air moisture. The affinity to acid dyestuffs for instance Alizarincyaningreen G Extra, Azoacidblack 3 BL Extra (Ullmann, Enzyklopaedie der technischen Chemie, second edition, vol. II, page 47) is enhanced.

I claim:

1. A method of improving the affinity to acid dyestuffs of artificial textile materials consisting chiefly of organic cellulose esters soluble in organic solvents and containing basic reacting groups, which method comprises reacting said textile materials before dyeing with a compound selected from the group consisting of alkylene-oxides, alkyleneimines and alkylenesulfides.

2. A method of improving the affinity to acid dyestuffs of artificial textile materials consisting chiefly of organic cellulose esters containing basic nitrogen, said cellulose esters being soluble in organic solvents, which method comprises reacting said textile materials before dyeing with a compound selected from the group consisting of

alkyleneoxides, alkyleneimines and alkylenesulfides.

3. A method of improving the affinity to acid dyestuffs of artificial textile materials consisting chiefly of organic cellulose esters soluble in organic solvents and having incorporated and fixed therein as an additional component a basic artificial resin which method comprises reacting the textile materials before dyeing with a compound selected from the group consisting of alkylene-oxides, alkyleneimines and alkylenesulfides.

4. A method of improving the affinity to acid dyestuffs of artificial textile materials consisting chiefly of organic cellulose acetate having incorporated and fixed therein a basic artificial resin which method comprises reacting said textile materials before dyeing with a compound selected from the group consisting of alkyleneoxides, alkyleneimines and alkylenesulfides.

5. Textile materials consisting chiefly of organic esters of cellulose and containing hydroxy alkylated basic nitrogen atoms, said materials being prepared by reacting artificial textile materials consisting chiefly of organic cellulose esters containing basic nitrogen with alkylene oxides.

PAUL SCHLACK.